

June 13, 1944.

W. J. FARRELL

2,351,415

GRID SUPPORT

Filed Feb. 2, 1943



FIG. 1



FIG. 2  
RATE OF WEIGHT LOSS  
BY METAL TEST PIECES  
IN AMMONIA OXIDATION UNITS

INVENTOR.  
William J. Farrell

BY

Claud and B. Adelbaugh  
ATTORNEY

## UNITED STATES PATENT OFFICE

2,351,415

## GRID SUPPORT

William J. Farrell, Parlin, N. J., assignor to Hercules Powder Company, Wilmington, Del., a corporation of Delaware

Application February 2, 1943, Serial No. 474,436

3 Claims. (Cl. 23—288)

This invention relates to the use of particular alloys in the construction of a grid support for the catalyst gauze used in the manufacture of nitric acid by the ammonia oxidation process.

The conversion of ammonia to nitric acid is carried out at a temperature of about 900 to 950° C. by passing a mixture of ammonia and air through a catalyst consisting of a number of layers of a catalyst gauze, such as platinum-rhodium gauze. The gauze is supported horizontally on a circular metal grid which in many installations is about 14 inches in diameter. The perimeter of the metal grid rests on a ledge on the inside of the oxidation unit at a point near the top. The grid is usually constructed in two halves. At the high temperature to which it is exposed, the grid deteriorates and buckles in time requiring frequent replacements to insure that the catalyst gauze may lie flat and the gas mixture pass entirely through it.

Many attempts have been made in the past to make this grid support of an alloy which is particularly resistant to deterioration under the particular conditions of the ammonia oxidation process. Examples of such alloys which have been used include chrome steels such as 18 chrome-8 nickel and 25 chrome-20 nickel; nickel-molybdenum-iron alloy of about a 62-30-5 parts ratio; nickel-molybdenum-chrome-iron alloy of about a 58-17-15-6 parts ratio; and cast alloy composed primarily of nickel and silicon plus small amounts of other catalytic elements. These have all been found to deteriorate or buckle badly in a relatively short time (3 to 4 months).

Now in accordance with the present invention, it has been found that a catalyst grid support of high resistance to deterioration may be made of an alloy comprising cobalt, chromium and tungsten in about a 55-33-6 parts ratio. This alloy is known to the trade as "Stellite 6" and is manufactured by the Haynes-Stellite Company.

Having indicated in a general way the nature and purpose of the invention, there follows a more detailed description of preferred embodiments thereof with reference to the accompanying drawing in which is shown in Figure 1 a perspective view of a typical circular grid catalyst support commonly used in the manufacture of nitric acid by the ammonia oxidation process. The catalyst support usually comprises two halves, the circumference of which is cast in separated portions. The circumferential portions are held together by reinforcing bars sufficiently separated to allow the passage of the gas and

forming a convex surface on one side of the support and a flat surface on the other.

The graph shown in the drawing at Figure 2 illustrates a comparison between various composition resistant alloys which have been tested and the cobalt-chrome-tungsten alloy of the present invention. In the graph, the per cent loss in weight is plotted against the number of hours that the sample of the alloy was exposed to the ammonia oxidation conditions. From the graph, it will be seen that the cobalt-chrome-tungsten alloy of the present invention is highly superior to any of the others shown, having, for instance, lost 0.5% of its weight after over 2000 hours of exposure to the ammonia oxidation conditions. It will be seen that the next base alloy tested, that is, chrome-nickel (25-20) steel loses over 3% or more than six times as much of its weight under the same conditions.

20 The following are the experiments results upon which the graph was based and serves to demonstrate the definite and unexpected superiority of the cobalt-chromium-tungsten alloy of the present invention:

|    |                                                               | Hours in service                                                                                                                                                                                                                                                      | Per cent weight loss                                                                                                                                                                                                                                                    |
|----|---------------------------------------------------------------|-----------------------------------------------------------------------------------------------------------------------------------------------------------------------------------------------------------------------------------------------------------------------|-------------------------------------------------------------------------------------------------------------------------------------------------------------------------------------------------------------------------------------------------------------------------|
| 30 | Nickel-molybdenum-iron alloy (62-30-5 parts ratio)            | 281<br>324<br>324<br>626<br>907<br>1,699<br>324<br>626<br>907<br>1,699<br>604<br>863<br>1,511<br>1,770<br>2,072<br>2,396<br>324<br>626<br>907<br>1,699<br>2,304<br>2,753<br>3,212<br>302<br>604<br>863<br>1,511<br>1,770<br>2,072<br>2,396<br>3,001<br>3,455<br>3,909 | 8.50<br>8.60<br>2.64<br>5.27<br>10.00<br>19.52<br>0.69<br>2.74<br>6.34<br>15.58<br>0.45<br>0.82<br>3.21<br>4.70<br>6.51<br>9.04<br>0.23<br>0.57<br>1.44<br>3.14<br>5.31<br>6.75<br>7.76<br>0.02<br>0.02<br>0.02<br>0.07<br>0.12<br>0.94<br>1.24<br>1.62<br>2.13<br>2.28 |
| 35 | Nickel-molybdenum-chrome-iron alloy (58-17-15-6 parts ratio)  |                                                                                                                                                                                                                                                                       |                                                                                                                                                                                                                                                                         |
| 40 | Cobalt-chromium-tungsten-iron alloy (30-30-10-20 parts ratio) |                                                                                                                                                                                                                                                                       |                                                                                                                                                                                                                                                                         |
| 45 | Chrome-nickel (25-20 parts ratio) steel                       |                                                                                                                                                                                                                                                                       |                                                                                                                                                                                                                                                                         |
| 50 | Cobalt-chrome-tungsten (55-33-6 parts ratio)                  |                                                                                                                                                                                                                                                                       |                                                                                                                                                                                                                                                                         |

While the particular alloy of the present invention has been described above as cobalt-chrome-tungsten (55-33-6 parts ratio), the alloy is that

which is known to the trade as "Stellite 6," a product of the Haynes-Stellite Company. The exact composition is not disclosed by the Haynes-Stellite Company, but it is a composition reasonably equivalent to that described above. Besides the above description, it is known that the composition is substantially free of iron.

Thus, the present invention has described a new and useful alloy which comprises cobalt-chrome-tungsten in about a 55-33-6 weight ratio which when used in the construction of a grid support for the catalyst in an ammonia oxidation converter has an excellent resistance to deterioration.

What I claim and desire to protect by Letters Patent is:

1. In an ammonia oxidation converter, a com-

bination of a wire gauze catalyst suitable for ammonia oxidation mounted on a grid support comprising a cobalt-chrome-tungsten alloy substantially free of iron.

5 2. In an ammonia oxidation converter, a combination of a wire gauze catalyst suitable for ammonia oxidation mounted on a grid support comprising a cobalt-chrome-tungsten alloy in about a 55-33-6 weight ratio, said alloy being substantially iron free.

10 3. In an ammonia oxidation converter, a combination of a wire gauze catalyst suitable for ammonia oxidation mounted on a grid support comprising two semicircular grids of a cobalt-chrome-tungsten alloy in about a 55-33-6 weight ratio, said alloy being substantially iron free.

WILLIAM J. FARRELL.